

June 30, 1953

J. ROCKOFF

2,643,436

SLASHER ROLL

Filed Aug. 15, 1949



Fig. 2

INVENTOR.  
JOSEPH ROCKOFF

BY  
*Joseph Rockoff*  
HIS ATTORNEY

## UNITED STATES PATENT OFFICE

2,643,436

## SLASHER ROLL

Joseph Rockoff, Dayton, Ohio, assignor to The  
Dayton Rubber Company, a corporation of  
Ohio

Application August 15, 1949, Serial No. 110,304

10 Claims. (Cl. 28—28)

1

This invention relates to an apparatus for the impregnation of textile materials and more particularly to an apparatus for the application of sizing to textile yarns in the operation known as slashing. This invention relates further to a novel type of roll especially adapted for use in the slashing operation.

Slashing is an operation used in the textile industry in the application of sizing material to textile fibers and yarns and in particular to cotton, rayon, and artificial silk fibers. Various types of sizing materials are used depending on the type of yarn and the results desired. Starches are generally used in the sizing of cotton yarns; whereas gelatine, soluble starches, and natural gums are most generally used in the sizing of rayon yarns. The sizing material may also include softeners, such as sulphonated oils, and penetrants or wetting out agents. The application of size to the textile yarn makes the yarn smoother and stronger to stand the strain of weaving, eliminates fraying, and facilitates subsequent handling of the yarn.

In carrying out the slashing operation, a number of strands of the work yarn are conveyed in parallel between one or more pairs of horizontal rollers usually arranged with a bottom roll at least partially immersed in the sizing liquid and a top roll resting on the bottom roll and driven by the rotation thereof. The yarn may pass between the rolls without immersion in the bath, thus being impregnated by the sizing liquid carried into contact with it by the bottom roller, or in some cases, may pass beneath the bottom roller for immersion in the sizing liquid prior to passing between the two rollers. The bottom rollers are generally made of copper and are gear driven. The top rolls, commonly known as the slasher rolls, are generally constructed of cast iron and are of considerable weight, usually weighing from 500 to 700 lbs. each. These are normally covered with resilient wool blankets. The function of the wool blanket, by the nature of its resilience and absorptive properties, is to remove excess size from the yarn as it emerges from the bite of the rollers. These blankets possess the necessary resilience and absorptive characteristics to properly dress the yarn to a predetermined proportion of sizing. In the case of cotton yarns using starch size, this usually runs to about 16% to 18% based on the weight of the yarn. In general, the slasher roll must have the property of uniformly distributing the size and controlling the proportion which is permitted to remain in the yarn, and must minimize the waste of excess

2

sizing material. Furthermore, the roll surface must be resistant to hot size solutions, such as, boiling starch, and must also be resistant to oils and chemicals which may be incorporated with the sizing material. In addition, the roll must eliminate flattening of the yarn and leave no roll marks, and must uniformly retain its resilience and absorptiveness over its period of use.

The wool blanket performs its operation satisfactorily but has the disadvantage of cost and short life in service. Attempts have been made to substitute for the wool blanket rolls covered with other materials, including synthetic rubber and the like, have been tried. Such attempts have been only partially successful since such roll surfaces, while more durable than wool, have not equalled or exceeded its adaptability to the sizing of various types of yarn using various types of sizing material.

10 It is therefore an object of the present invention to provide an apparatus for the impregnation of textile materials with size or the like in which the roll surface shall be durable and at the same time adaptable to a wide range of conditions.

15 It is a further object of the present invention to provide a slashing roll having a surface structure which is highly resistant to the sizing material and to the conditions of operation over a long period of time and which will at the same time properly dress the yarn to a predetermined concentration of size.

20 In accordance with the present invention it has been found that an apparatus of the type described may be constructed using rolls having rubber containing surfaces which will function over a wide range of conditions to produce sized yarns containing predetermined proportions of sizing material. The result is obtained by forming the slasher roll with a surface composition of rubber having incorporated therein or admixed therewith a desired proportion of wool fibers. The wool-rubber composition is prepared by milling into the rubber the desired proportion of wool fibers. Usually wool waste containing fibers ranging in length from  $\frac{1}{16}$ " to  $\frac{1}{2}$ " is satisfactory for the purpose. The proportion of fibers incorporated with the rubber is variable and will depend upon the particular conditions involved. In general, it is preferred to utilize substantial proportions of wool fiber and it has been found that an optimum range is from 100 to 200 parts of wool fiber by weight for each 100 parts of rubber hydrocarbon by weight.

25 30 35 40 45 50 55 60 65 70 75 80 85 90 95 The term "rubber" as used herein is intended

to include both natural and synthetic rubbers. By the term "synthetic rubbers" is meant the synthetic elastomers having the properties of resilience, elasticity, and vulcanizability similar to those possessed by natural rubber. The synthetic rubbers in general include the rubber-like polymers of conjugated diolefins and their copolymers with styrene, acrylic nitrile, and other monomers known to be copolymerizable therewith. The synthetic rubbers also include the chloroprene polymers known as neoprene, the iso-olefin diolefin copolymers known as butyl rubber, and the polysulfide polymers known as Thiokol. In applications where the rolls are exposed to extreme conditions of temperature, oils, and the like, it is preferred to use the oil resistant types of synthetic rubber, such as neoprene, and the butadiene-acrylic nitrile copolymers, such as Hycar OR, and/or Buna-N.

The slasher rolls may be composed entirely of the rubber-wool composition mounted on an arbor shaft, but generally it is preferred to utilize this composition only as the roll surfacing material with the rest of the roll preferably constituted of wool-free rubber of any desired type.

The invention will be more fully understood from the description of the accompanying drawings which illustrate a typical arrangement for the sizing of cotton yarns together with a typical construction of a slasher roll adapted for this purpose and constructed in accordance with the present invention.

In the drawings:

Fig. 1 is a side elevational view partly in cross section of an apparatus incorporating the novel features of the invention.

Fig. 2 is a cross sectional view partly in elevation taken along lines 2—2 of Fig. 1.

Fig. 3 is an enlarged fragmentary cross sectional view taken along line 3—3 of Fig. 2.

Referring to the drawings in detail, reference numeral 10 as shown in Figs. 1 and 2 indicates a container for holding sizing bath 11. Thread or yarn to be sized is designated by reference numeral 12. This material is guided between a front drive roll 13 and a back drive roll 14 both made of steel and mounted near the top of the bath so as to be partially submerged therein. Both of these rolls are driven by shaft 24 through beveled gears 25 and 26. Above each of the lower rolls 13 and 14 is mounted a rubber covered slasher roll. These rolls are designated by reference numerals 15 and 16. These rolls run freely driven by the friction of their weight resting on the rotating bottom rolls. The slasher rolls are mounted in bearing blocks 21 vertically slidable in U shape slots 22 which are formed in end bearing brackets 23. These slots are open at the top to facilitate removal of the rolls for cleaning, and permit the full weight of rolls 15 and 16 to bear upon the thread 12. Although Figs. 1 to 3 show the yarn or thread as keeping the top and bottom rolls slightly apart, this is for the purpose of illustration only since in actual practice the surfaces of the slasher rolls are sufficiently resilient so that they are in rolling contact with the bottom rolls with the thread or yarn in between.

Each slasher roll 15 and 16 comprises a layer of the desired wool fiber-rubber composition 17 on the surface, preferably cemented to or otherwise secured to an intermediate rubber layer 18 which is in turn mounted upon a shaft or arbor 19. If desired, the entire rubber portion of the roll may be constructed of the wool-rubber composition, or the intermediate layer 18 of rubber

may be omitted and replaced by a synthetic resin composition, or by metal, or any other desired material.

Fig. 3 illustrates a cross section of a surface portion of the slasher roll showing the wool fiber-rubber composition 17 in contact with the yarn 12. As shown, the wool fibers are dispersed in random fashion in the rubber.

A typical compound used in making rolls of the present invention is as follows:

|                                           | Parts by weight |
|-------------------------------------------|-----------------|
| Butadiene acrylonitrile copolymer (Hycar) | 100             |
| Zinc oxide                                | 10              |
| Sulfur                                    | 2               |
| Accelerator                               | 1               |
| Whiting                                   | 50              |
| Stearic acid                              | 2               |
| Wool fiber                                | 100             |
| Softener                                  | 10              |

A pair of slasher rolls was fabricated having the following dimensions: core 6 $\frac{5}{8}$ " diameter; finished roll 8 $\frac{5}{8}$ " diameter, 58" in length. The core was covered with a layer of oil-resistant butadiene acrylic nitrile copolymer about  $\frac{1}{8}$ " in thickness. This intermediate layer was then covered with a sleeve composed of the same type of rubber  $\frac{1}{8}$ " in thickness but containing 100 parts of ground up wool fibers for each 100 parts of rubber. This sleeve was adhered by means of cement to the intermediate layer. The rolls were then utilized in the slashing of cotton yarn in a sizing bath containing starch, tallow, emulsifying oils, natural gum, and water, operated at 212° F. These rolls were operated continuously for a period of four months and gave perfectly satisfactory performance during that period. At the end of that time the rolls were examined and found to show some slight signs of wear. The surface of each roll was then buffed and working surfaces as good as that of the original roll were obtained. The rebuffed rolls were then placed in operation and after an additional period of four months were still functioning satisfactorily. A pair of conventional metal rolls covered with wool blankets operating with the same kind of sizing bath upon the same type of yarn, operated satisfactorily only for a period of about four weeks and could not be renewed or reused since a new covering had to be applied to the cores. This clearly demonstrates that the wool fiber-rubber composition performed as well as the wool blanket covered rolls but possessed strikingly greater durability since the rolls could be used almost indefinitely with occasional rebuffing.

While certain specific embodiments of the invention have been described herein, it is not intended that it shall be limited thereto and the invention is susceptible to various modifications and changes which come within the spirit of this disclosure and the scope of the appended claims.

I claim:

1. A slasher roll for the controlled application of sizing material to textile fibers and yarns in textile sizing machines which comprises a surface layer of milled rubber having a substantial proportion of wool fibers intimately dispersed therein.

2. A slasher roll according to claim 1 wherein the wool fibers are in the proportion of one to two parts by weight of the wool for each part by weight of the rubber.

3. A slasher roll according to claim 2 wherein the wool fibers have a length within the range of  $\frac{1}{16}$ " to  $\frac{1}{2}$ ".

4. A slasher roll according to claim 1 wherein the rubber is natural rubber.

5. A slasher roll according to claim 1 wherein the rubber is synthetic rubber-like material.

6. A slasher roll according to claim 5 wherein the synthetic rubber-like material comprises a butadiene-acrylonitrile copolymer.

7. A slasher roll according to claim 1 wherein the rubber is a synthetic rubber-like material comprising a chloroprene polymer.

8. A slasher roll for the controlled application of sizing material to textile fibers and yarns in textile sizing machines which comprises a metal core, an intermediate layer of rubber free from wool fiber, and a surface layer of milled rubber comprising a substantial proportion of wool fibers intimately dispersed therein.

9. An apparatus for the application of textile sizing liquids to textile materials comprising a liquid bath, a guide roll at least partially submerged in said bath for conveying textile materials therethrough, a rubber covered roll positioned above said guide roll exteriorly of the bath and resting thereon, means for passing textile material between said rubber covered roll and

10

20

25

said guide roll, said rubber covered roll having a surface composed of milled rubber having a substantial proportion of wool fibers intimately dispersed therein.

10. An apparatus according to claim 9 wherein the surface of the roll has incorporated therein from 100 to 200 parts of wool fiber for each 100 parts of rubber.

JOSEPH ROCKOFF.

References Cited in the file of this patent

UNITED STATES PATENTS

| Number    | Name       | Date          |
|-----------|------------|---------------|
| 1,628,261 | McGann     | May 10, 1927  |
| 2,108,189 | Batchelder | Feb. 15, 1933 |
| 2,150,178 | Maywald    | Mar. 14, 1939 |
| 2,207,932 | Morrison   | July 16, 1940 |
| 2,393,953 | Bacon      | Feb. 5, 1946  |
| 2,426,227 | Luaces     | Aug. 26, 1947 |
| 2,507,869 | Rothermel  | May 16, 1950  |

FOREIGN PATENTS

| Number  | Country       | Date          |
|---------|---------------|---------------|
| 254,866 | Great Britain | July 15, 1926 |